

3,165,401

**ALLOY STEEL FOR CAST PARTS RESISTANT TO HIGH TEMPERATURES AND CORROSION**  
Emil Reusch, Fort Wayne, Ind., assignor to International Harvester Company, Chicago, Ill., a corporation of New Jersey  
No Drawing. Filed Mar. 20, 1957, Ser. No. 647,216  
10 Claims. (Cl. 75—128)

This invention relates to a new and improved stainless steel, and more particularly to a steel suitable for the casting of internal combustion engine parts, valves and the like, gas turbine parts, etc., which must possess qualities of high strength, high hardness, and high resistance to corrosion oxidation and scaling at elevated temperatures. In the effort of increasing the output of internal combustion engines the trend has constantly been to higher operating temperatures. To avoid certain undesirable results of such increased temperatures it has been necessary to add to the fuel, anti-detonants which, however, greatly increase the corrosive effects on parts which come into contact with the products of combustion. In the conventional internal combustion engine, one of these parts which is seriously affected is the engine exhaust valve. The materials heretofore used have proven to be unsatisfactory in meeting the aforementioned conditions prevalent in present day higher efficiency engines. Exhaust valves made from conventional materials, forged or extruded, usually stretched over their whole length, cupped in the head portion and cracked at the stem close to the head of the valve, which failures in many instances occurred as a direct result of the high temperatures and the lack of the material to withstand the effect of the forces acting on the valve. The increase of the corrosive effect showed up mainly in eating away the material in the neck portion and on the outer rim of the valve. It is a fact, therefore, that a good valve material that will meet present day requirements must possess the following characteristics: high hot hardness, high hot strength, good wear resistance, high creep resistance, low thermal expansion; high shock resistance, low ductility, high toughness, high oxidation and corrosion resistance, high thermal conductivity and good scaling resistance.

Valves heretofore made by the process of forging or extruding (known as wrought valves) have been observed to more readily stretch, during operation, to the breaking point or generally become quickly brittle resulting in premature failures due to cracking or distorting of the rim of the valve head. In addition to the inadequacies of the material utilized it is also apparent that such failures are further abetted by the forging or extruding techniques which generally limits the chemical composition and sets up undesirable grain patterns in the finished product.

It is a prime object of this invention therefore to provide an improved alloy steel having chemical properties ideally suited for casting, to provide manufactured parts having inherent resistance characteristics with respect to high temperatures and products of combustion resulting from the operation of an internal combustion engine.

A still further object is to provide an improved material particularly suited to the manufacture and use of an improved cast valve.

Another object is to provide an improved stainless steel having a chemical combination which particularly meets, to a maximum degree, all of the desirable characteristics of a valve element as expressed above.

A more specific object is to provide an improved alloy steel particularly suited to parts subjected to the conditions and products of combustion of an engine, the material having among other things a silicon content which

particularly suits the same to the manufacture of cast parts, such as exhaust valves, etc.

A further object is to provide a steel alloy material particularly suited to cast parts subjected to high temperatures and corrosion, the material having favorable work hardening characteristics which improve the inherently favorable characteristic of the cast article during use.

In the development of the improved cast alloy steel certain resultant factors have been taken into consideration. Chromium is of course particularly desirable in that it provides high corrosion resistance. Up to 25% chromium may be particularly beneficial in this respect but over this figure brittleness generally results. Applicant's steel therefore utilizes a chromium range of approximately 20 to 22% which assures high corrosive resistance without the possible undesirable characteristics which additional chromium might produce. Carbon of course will increase the hardness of an austenitic structure but it also may, when united with chromium increase the susceptibility to corrosion. This results when the carbon at higher temperatures becomes unstable and is rejected from solid solutions in the form of chromium-rich carbide. Thus adjacent areas of the metal become impoverished in chromium with resultant increase in corrosion. In the present material a range of .90% to 1.20% carbon has been found to be particularly effective.

The important characteristics of hot hardness and hot strength are not found in predominantly chromium-iron-carbon alloys and in addition therefore an austenizing element is necessary where the aforesaid properties are of pronounced importance. Nickel is a well known element for this purpose. Nickel may however have an adverse effect on corrosion resistance while operating in the presence of lead compounds of amounts required for improved engine operation. Furthermore nickel is of course also a very scarce product. By supplanting a substantial quantity of nickel ordinarily required for austenitic quality, with manganese, an austenitic steel is obtained and the adverse effect of nickel upon corrosion resistance in the combustion products of leaded fuels is largely dispelled. Accordingly in my alloy steel the nickel content is reduced to the smallest percentage 1.00% to 2%.

Manganese has been substituted for larger proportions of nickel. It contributes markedly to strength and hardness and tends to decrease the critical cooling rate of the material. Further with increasing carbon lower ductility results. Manganese being highly resistant to sulphur and lead bearing atmospheres is also very desirable. In my alloy I utilize a manganese content of 5.00% to 8.00%. Above this figure a possibility exists of delta ferrite formation and resultant brittleness.

Nitrogen contributes greatly to hot strength and toughness in my material as well as serving to retain the austenitic structure under the combined action of thermal and mechanical forces. This material in combination with manganese substitutes for my decrease in the nickel content. It further restricts grain growth while maintaining its important characteristic of being an austenizing element. The chromium and manganese of my material increase the solubility of the nitrogen which exists in the range of .20% to 0.40%.

Wrought steel alloys normally contain less than .50% silicon. This is particularly true of a conventional valve material where the silicon content is held below .25%. With a low silicon content of this type the advantages of a cast material cannot be obtained. High silicon content is important in promoting castability of my alloy. Too low a silicon content will also result in poor weldability and poor scaling resistance. Too high a silicon content may cause serious brittleness. In our cast valve material I have adapted a range of .60% to 1.20% silicon

to obtain with the high carbon, high hot hardness and a high degree of scale resistance without adversely affecting the corrosion resistance. Furthermore the high silicon also provided better castability of the material.

The steel then consists of the following:

|           | Percent        |
|-----------|----------------|
| Carbon    | 0.90 to 1.20   |
| Silicon   | 0.60 to 1.20   |
| Manganese | 5.00 to 8.00   |
| Chromium  | 15.00 to 25.00 |
| Nickel    | 1.00 to 2.00   |
| Nitrogen  | 0.20 to 0.40   |
| Iron      | Balance        |

Some of the properties of this material in the "as cast" condition are as follows:

| Tensile Properties                                        | Room Temp. | 1,000° F. | 1,200° F. | 1,400° F. | 1,500° F. | 1,600° F. |
|-----------------------------------------------------------|------------|-----------|-----------|-----------|-----------|-----------|
| Ultimate Strength, p.s.i.                                 |            | 106,650   | 76,150    | 66,850    | 52,400    | 44,300    |
| Yield Strength (.2%) p.s.i.                               |            | 86,500    | 56,100    | 50,000    | 44,900    | 37,500    |
| Elongation, - Percent in 4D                               |            | 4.29      | 5.72      | 5.72      | 4.75      | 4.6       |
| Reduction of Area, - percent                              |            | 3.39      | 5.61      | 6.12      | 5.82      | 7.21      |
| Hardness after test At Room Temperature (R "C")           | 28.6       | 29.5      | 29.5      | 35.2      | 39.4      | 37.4      |
| Hardness                                                  | Room Temp. | 1,000° F. | 1,200° F. | 1,400° F. | 1,500° F. | 1,600° F. |
| Brinell (750 Kg. - 5 mm. Ball), At different temperatures | 289        | 212       | 173       | 159       | 132       | 89        |
| Hardness after test At Room Temperature (R "C")           | 31         | 32        | 31.2      | 35        | 39        | 39.5      |

As indicated in my stated objects my improved material is particularly adapted for casting and thus grain structure advantages can be achieved which are not possible in forged or extruded (wrought) materials. A wrought valve for instance stretches and distorts in the rim portion which leads to burning or it becomes brittle and breaks under the high temperature condition. It is believed that this undesirable condition, in addition to conventional materials used, results from the grain structure obtained incident to the forging or extruding operation.

Grains in cast material are very coarse by wrought material standards. Coarse grain size, however, is beneficial since most failures are intergranular, and coarse grained materials, having less grain boundary, are less prone to intergranular failure. This is of particular importance in my valve material since this material is operating at high temperature at which the grain boundaries generally become weaker and failure more likely will result. Furthermore it has become apparent that stress orientation in the crystal structure of a cast valve is considerably more favorable to the conditions to which it is subjected than in a forged valve. The present material therefore is particularly suited for casting. While it is especially adapted for exhaust valves it must be realized that it has particular adaptability for any parts which must operate at high temperature and under conditions where hot corrosive gases are incident to the operation.

Another desirable feature of my material is its hardenability. It is capable of work and age hardening to over 40 Rockwell "C." On quenching from 2150° F. it has a hardness of about 30 Rockwell "C" and on reheating to 1400° F. and holding it there for 8 hours, its hardness increases to 42 to 45 Rockwell "C" hardness.

The terms above, namely, "work and age hardening" have particular significance in the present valve steel. The cast valve herein described is placed into the engine in the as-cast condition without hardening by precipitation or by other means. During the use in the engine significant changes taken place in valve and it is felt that these changes are a result of a combination of work

and age hardening. The valve in the engine is repeatedly heated and cooled which to a great extent no doubt transforms the structure of the material in the same way that results from age hardening. In addition, however, certain structural changes take place in the valve which also are believed to definitely result from the phenomenon of work hardening. Not only does the valve develop greater hardness but also the mechanical properties are definitely improved and it is felt that this is due to the steady impounding and the state of stress under which the valve works in the engine. In other words this material consistently improves during the operation of the engine whereas other valve materials known in the art deteriorate during operation. High hardness increases the amount of elastic deformation that can be tolerated. The combination of high hardness with low

modulus will result in superior wear resistance of the material. In determining the best suited elastic modulus and the higher possible hardness, my material composition was chosen to have low atomic weight sum and high melting temperature. In this respect my casting material shows a great difference when compared with the commercially available valve materials (wrought materials).

Another important feature of this material is its work hardening ability. Hardness of the cast material is not diminished due to elevated operating temperatures but in contradiction, it is increased due to work-hardening. Thus a valve made from my material may go into an engine at 30 Rockwell "C" and during operation in the engine the Rockwell hardness increases from 30 to 41-45 RC.

Thus, it is readily apparent that the objects of the invention have been fully achieved. Changes and modifications in the composition may be made which do not depart from the spirit of the invention, or from the scope of the appended claims.

What is claimed is:

1. A stainless steel having high resistance to high temperatures and products of internal combustion, containing about 0.90% to 1.20% carbon, about 0.60% to 1.00% silicon, 5% to 8% manganese, 20% to 22% chromium, 1% to 2% nickel, about 0.20% to 0.40% nitrogen, and the remainder substantially iron.

2. A stainless steel valve having high resistance to high temperatures and products of internal combustion, containing about 0.90% to 1.20% carbon, at least 0.60% to 1.00% silicon, 5% to 8% manganese, 20% to 22% chromium, 1% to 2% nickel, about 0.20% to 0.40% nitrogen, and the remainder substantially iron.

3. A stainless steel having high resistance to high temperatures and products of internal combustion, containing about 0.90% to 1.20% carbon, at least 0.60% to 1.20% silicon, 5% to 8% manganese, 20% to 22% chromium, 1% to 2% nickel, about 0.20% to 0.40% nitrogen, and the remainder substantially iron.

4. A stainless steel material particularly adapted for casting internal combustion engine valves which during

use are subjected to high temperatures and corrosive atmospheres containing about 0.90% to 1.20% carbon, 0.60% to 1.20% silicon, about 5% to 8% manganese, 20% to 25% chromium, 1% to 2% nickel, 0.20% to 0.40% nitrogen, and the remainder substantially iron.

5. A stainless steel material particularly adapted for casting internal combustion engine valves which during use are subjected to high temperatures and corrosive atmospheres containing about 0.90% to 1.20% carbon, 0.60% to 1.20% silicon, about 5% to 8% manganese, 15% to 22% chromium, 1% to 2% nickel, 0.20% to 0.40% nitrogen, and the remainder substantially iron.

6. A stainless steel material particularly adapted for casting parts which during use are subjected to high temperatures and corrosive atmospheres containing about 0.90% to 1.60% carbon, not less than 0.60% and not more than 1.20% silicon, about 5% to 8% manganese, 20% to 25% chromium, not less than 1% and not exceeding 2% nickel, 0.20% to 0.40% nitrogen, and the remainder substantially iron.

7. A stainless steel material for producing cast internal combustion engine valves containing not less than 0.90% and not more than 1.20% carbon, about 0.60% to 1.00% silicon, 5% to 8% manganese, 15% to 25% chromium, 1% to 2% nickel, 0.20% to 0.40% nitrogen, and the remainder substantially iron.

8. An austenitic stainless steel consisting essentially of about 0.90% to 1.50% carbon, 0.60% to 1.20% silicon, 5% to 8% manganese, 15% to 25% chromium, 1% to 30

2% nickel, 0.20% to 0.40% nitrogen and the remainder substantially all iron.

9. An austenitic alloy consisting essentially of about 0.9% to 1.0% carbon, 0.6% to 1.0% silicon, 5% to 8% manganese, 15% to 25% chromium, 1% to 2% nickel, 0.2% to 0.4% nitrogen and the remainder substantially iron.

10. An austenitic iron-base valve having high strength and hardness and good resistance to corrosion in the presence of leaded fuel combustion products at valve operating temperatures and containing as essential alloying elements carbon from about 0.9% to about 1.0%, manganese from about 5.0% to about 8.0% silicon from about 0.6% to about 1.20%, chromium from about 15.0% to about 25.0%, nickel from about 1.0% to about 2.0%, nitrogen from about 0.2% to about 0.4%, the balance being iron with incidental impurities.

#### References Cited in the file of this patent

20

#### UNITED STATES PATENTS

|           |                |               |
|-----------|----------------|---------------|
| 2,015,991 | Breeler        | Oct. 1, 1935  |
| 2,225,440 | Becket et al.  | Dec. 17, 1940 |
| 2,380,821 | Breeler et al. | July 31, 1945 |
| 2,496,247 | Jennings       | Jan. 31, 1950 |
| 2,602,738 | Jennings       | July 8, 1952  |
| 2,706,696 | Payson         | Apr. 19, 1955 |
| 2,768,918 | Armstrong      | Oct. 30, 1956 |

#### FOREIGN PATENTS

Great Britain ----- Apr. 15, 1929